

## UNITED STATES PATENT OFFICE

2,352,922

## PAPER MANUFACTURE

Joseph J. Thomas, Springfield, Mass., Robert A. Diehm, Appleton, Wis., and Ian C. Somerville, Philadelphia, Pa., assignors to Röhm & Haas Company, Philadelphia, Pa.

No Drawing. Application October 6, 1939,  
Serial No. 298,340

6 Claims. (Cl. 92—21)

This invention relates to improved methods in the manufacture of paper, whereby the retention of filler is increased, sizing is improved, and sheets of improved uniformity and texture and of high wet strength are obtained. In particular it deals with the precipitation and dispersion of sizes, particularly of protein sizes, among paper fibers by a procedure involving the use of syntans.

Glue and casein are often used for the tub sizing and coating of paper, but their use as sizing materials in the beater for treating pulp which is to be formed into paper sheets has not been practical. The agents for precipitating proteins, previously available, have not been applied successfully for sizing in the beater. While the hardening of glue applied in a tub-sizing operation has been accomplished by formaldehyde, it has not been practical or economical to mix glue and formaldehyde with pulp. When formaldehyde is added to the beater, it appears to be too dilute to be effective or it insolubilizes a glue size in such a way that the size is of little value. While aluminum salts are successfully used to precipitate rosin, they likewise have been ineffective in glue sizing. It has also been proposed to precipitate proteins with tannic acid, but this reaction has not produced the desired results in beater-sizing and suffers from other disadvantages, such as color. Agents heretofore available for fixing glue and other proteins have been ineffective in warm or hot solutions. While the agents mentioned have been found useful in some particular phase of paper-making, they have not been of more general application and have not permitted the improvements which have now been found possible.

An object of this invention is to provide a method for preparing paper of improved wet strength. It is also an object to utilize in an improved manner proteins, particularly glues, for the beater sizing of paper. It is a further object to prepare paper which possesses not only high wet strength, but high dry strength, and which is pervious to moisture and can serve for the common uses of paper or for a paper base which may be further coated as for a glazed paper, or blueprint paper. It is also an object to prepare sized papers of improved properties, as shown by ink penetration and writing tests. It is a still further object to produce better formed sheets with increased utilization of fine fibers and better retention of solids, including fillers. It is also a further object to improve the dyeing of paper, including the dispersion of the dye-

stuff and its fixation. It is a further object to utilize protein sizing along with other sizing, such as rosin, improving the dispersion of the rosin, and ensuring even distribution of the rosin throughout the fibers and at the same time eliminate difficulties due to the presence of natural resins or pitch in the fibers or in the water.

These objects are accomplished by the application of a syntan along with a water-soluble protein in the treatment of cellulose fibers before they are formed into a paper sheet.

In preparing paper of superior properties by the use of a water-soluble or lyophilic protein and a syntan, these materials are mixed with cellulose fibers or pulp in water, usually in the beater. Rosin, color, and fillers may be added before or after the protein and syntan. When the stock has been worked to a satisfactory degree of freeness or the added materials thoroughly and uniformly incorporated, the pH of the suspension is adjusted so that it is at about, or below, the isoelectric point of the lyophilic protein which is used. The most commonly used material for lowering the pH to about the isoelectric point is alum. When the proper pH is reached, the protein is precipitated on the fibers, which are then formed into a sheet, which is, in turn, finished in the usual way for the particular type of paper at hand.

The order of addition of the various materials, pulp, protein, rosin, syntan, coloring material, filler, etc., may be widely varied. If the furnish stock is neutral or slightly alkaline, it may be adjusted to a slightly acid condition by the use of an acid syntan, other acid such as sulfuric acid, or alum. A pH of about 6 is entirely satisfactory for preventing foam when glue, gelatin, or other protein is used with a syntan. The amount of protein added may be varied from 0.2% to 5% of the dry weight of the furnish stock. The quantity of syntan used may be varied from 10% to 100% of the weight of the protein taken. It is preferred to dissolve the protein and the syntan separately and add the solution of each to the suspension of furnish stock, although the syntan and protein can be mixed in solution if the pH of the mixture is kept above the isoelectric point of the protein. Indeed, in the case of rag content papers where better sizing is needed, particularly during hot weather, it is preferable to mix the syntan and protein before dumping into the beater; or, if the beater has already been dropped, the glue-syntan can be added to the machine chest in order to restore sizing to the sheet. Starch or rosin size may be added and

beaten into the mix. Color and filler may also be added. The syntans act as dispersing agents for these materials and ensure uniform and even distribution of them throughout the pulp. The syntans also disperse pitch which may be present, particularly in mechanical or unbleached pulps, or gummy substances occurring in the water. If desired, the syntan, in whole or in part, may be added with the rosin size to help insure even distribution of the size and to prevent accumulation of size on the sides of the beater, in the valves, or in the pipe lines.

The pH of the mixture of pulp, size, filler, etc. is preferably adjusted to about the isoelectric point of the protein just before the suspension is to be formed into a sheet. This operation is best accomplished in the beater just before the charge is dropped to the chest. In the case of animal glues, usually from hoof, hide, or bone, the desired pH lies between 4.2 and 5.0, with a maximum of effectiveness at about 4.7.

There may be used in the place of animal glue any water-soluble, lyophilic, protein colloid such as albumen, gelatin, or even casein. The latter material, however, is somewhat more difficult to handle than the others since it must usually be dispersed with alkali and is less effective.

As syntans there may be used the wide variety of synthetic materials which have been developed and recognized in the leather industry for the fixation of hide substance. Typical examples are the formaldehyde condensates of naphthalene sulfonic acid, benzidine disulfonic acid, phenol sulfonic acids, such as 4,4'-dihydroxydiphenyl sulfone sulfonate, etc., the condensates of phenols with urea, thiourea, dicyandiamide, etc. and formaldehyde which are solubilized by sulfonation, reaction with naphthalene sulfonic acid, reaction with the formaldehyde condensate of naphthalene sulfonic acid, a phenol sulfonic acid, or the like. These materials are most conveniently applied in the form of their salts, which are obtained upon neutralization of the acid condensates. But partially neutralized materials may also be used and with proper care as to the adjustment of pH and with due regard to the nature of other materials added, fully acid materials may also be used, at least to some extent.

The process of forming paper from fibers with the addition of protein and a syntan results in many advantages. There is a high retention of fine cellulose fibers. The white water is clearer than in other processes. The syntans properly applied reduce greatly any difficulties due to foam. The sheet is better formed and more uniformly formed, probably due to a better filtering medium on the wire. In some cases it has been noted that the syntan gives an artificial slowness to the stock which undoubtedly helps account for more even distribution. The better formation of sheets tends to enhance most of the properties of the paper. For example, the paper exhibits increased toughness throughout the sheet as shown, for instance, by improved erasing qualities of drawing and ledger paper. The wet strength of syntan-prepared paper is improved. Rosin, used as a size, is more uniformly and evenly distributed and deposited. Other sizing materials are also more uniformly and effectively used when syntans are employed. The improvement in sizing is particularly noticeable in ink penetration and writing tests. Fillers are well dispersed, evenly distributed and well retained in the presence of syntans. When dyes are used, they are likewise dispersed and more efficiently utilized. Basic dyes appear to

be mordanted by the syntans. The presence of syntans in the beater also helps to disperse pitch when it happens to be present and thus prevents stains or holes in the finished sheets and clogging of screens or sticking on the cans.

The following examples are typical of procedures for improving the preparation of paper.

*Example 1.*—To approximately 40,000 lbs. of water in the beater are added 2,000 lbs. of cellulose fibers (half sulfite pulp and half ground wood). The pulp is beaten to the desired freeness and alum carefully added until the pH of the suspension is 6. There is then added a solution containing 10 lbs. of hide glue, followed by the addition of two pounds of the neutral sodium salt of the formaldehyde condensate of naphthalene sulfonic acid. After mixing has continued for a short time, a rosin emulsion equivalent to 40 lbs. of rosin is added followed by mineral filler to the extent of 100 lbs. When these materials have been well worked in, alum is added until a pH of 4.7 is reached. The beater is then dropped to the machine chest, water is added, and the suspension used for making paper in the usual way.

*Example 2.*—About 2500 lbs. of kraft pulp are beaten to the desired degree of freeness in approximately 50,000 lbs. of water. About 5 lbs. of the formaldehyde condensate of 4,4'-dihydroxydiphenyl sulfone sulfonate are added and 15 lbs. of animal glue which has been thoroughly soaked out and taken up in water. Filler, rosin, and color are then added and another pound of the syntan followed by sufficient alum to bring the pH below 4.7. The pulp was then dropped to the stuff-chest, diluted, formed into a sheet, and dried. The resulting paper had a high Mullen test.

*Example 3.*—A mixture of 1800 lbs. of sulfite pulp and 200 lbs. of gummed tape broke are beaten in about 38,000 lbs. of water. A neutral solution of 8 lbs. of the solubilized condensate of phenol sulfonic acid, urea, and formaldehyde is added, followed by 30 lbs. of rosin soap and 75 lbs. of clay. After the mixture is well beaten, about 30 lbs. of alum are added to bring the pH to about 4.6 and paper is formed in the usual way. Over 90% of the glue from the gummed tape is retained in the paper.

*Example 4.*—About 1500 pounds of rag stock (properly prepared by cooking, washing, etc.) are mixed in a beater with about 30,000 lbs. of water. The stock is beaten to the desired freeness. There is added a solution containing 8 lbs. of glue and 1.5 lbs. of syntan, the pH of which is above 4.7. This is followed by 30 lbs. of rosin soap, and mixing continued. Finally alum to a pH of 4.5 is added and the stock dropped to the chest from which it is flowed to the paper making machine. Improved writing qualities result from this treatment.

The protein-syntan prepared paper may be further sized or protein may be further insolubilized by the use of formaldehyde. This latter treatment is of particular value for the preparation of papers which must withstand soaking in water such as blueprint paper.

We claim:

1. The process of improving the uniformity, texture, and wet strength of paper and increasing the retention of filler therein, which comprises mixing with paper fibers suspended in water a water-soluble protein in an amount between 0.2% and about 5% of the dry weight of the paper fibers and a synthetic sulfonated aromatic compound, having tanning properties, in

an amount between about 10% and about 100% of the weight of said protein, incorporating filler in the resulting mixture, adjusting the pH thereof until it is lowered at least to about the isoelectric point of said protein, forming the mixture into a paper sheet, and drying said sheet.

2. The process of improving the uniformity, texture, and wet strength of paper and increasing the retention of filler therein, which comprises mixing with paper pulp in aqueous suspension animal glue in an amount between 0.2% and about 5% of the dry weight of the paper pulp and a synthetic sulfonated aromatic compound, having tanning properties, in an amount between about 10% and about 100% of the weight of the glue, incorporating filler with the pulp, adjusting the pH of the resulting mixture until it is lowered at least to about the isoelectric point of the glue, forming the mixture into a paper sheet, and drying said sheet.

3. The process of improving the uniformity, texture, and wet strength of paper and increasing the retention of filler therein which comprises mixing with paper pulp in aqueous suspension animal glue in an amount between 0.2% and about 5% of the dry weight of the paper pulp and a synthetic sulfonated aromatic compound having tanning properties, in an amount between about 10% and about 100% of the weight of the glue, incorporating filler with the pulp, adding alum to the resulting mixture until the pH thereof is brought at least to about the isoelectric point of the glue, forming the mixture into a paper sheet, and drying said sheet.

4. The process of improving the uniformity, texture, and wet strength of paper and increasing the retention of filler therein, which comprises mixing with paper pulp in aqueous suspension

5 animal glue in an amount between 0.2% and about 5% of the dry weight of the paper pulp and a water-soluble salt of a condensate of naphthalene sulfonic acid and formaldehyde in an amount between about 10% and about 100% of the weight of the glue, incorporating filler with the pulp, adding alum to the resulting mixture until the pH thereof is brought at least to about the isoelectric point of the glue, forming the mixture into a paper sheet, and drying said sheet.

10 5. In the process of making paper of high wet strength, the improvements which comprise mixing with an aqueous suspension of paper fibers animal glue in an amount between about 0.2% and about 5% of the dry weight of the paper fibers and the sodium salt of naphthalene sulfonic acid condensed with formaldehyde in an amount between about 10% and about 100% of the weight of the glue, and subsequently adding 15 alum to the aqueous suspension containing paper fibers, glue, and said sodium salt until the pH of said suspension is brought at least to about the isoelectric point of the glue.

20 6. In the process of making paper of high wet strength the improvements which comprise mixing with an aqueous suspension of paper fibers a water-soluble protein in an amount between 0.2% and about 5% of the weight of the paper fibers and a synthetic sulfonated aromatic compound having tanning properties in an amount between about 10% and about 100% of the weight of said protein, and subsequently adjusting the pH of said suspension at least to about the isoelectric point of the protein.

JOSEPH J. THOMAS.  
ROBERT A. DIEHM.  
IAN C. SOMERVILLE.